

Dec. 10, 1940.

W. J. BULLOCK

2,224,425

PROCESS OF RECOVERY OF PLATING METAL FROM SCRUFF

Filed Jan. 20, 1940



## UNITED STATES PATENT OFFICE

2,224,425

PROCESS OF RECOVERY OF PLATING  
METAL FROM SCRUFFWilliam J. Bullock, Birmingham, Ala., assignor to  
W. J. Bullock, Inc., a corporation of Delaware

Application January 20, 1940, Serial No. 314,886

2 Claims. (Cl. 75—64)

My invention relates to the recovery of plating metal from scruff such as is accumulated in sheet metal plating processes wherein the sheets are dipped into molten plating metal.

5 It is the principal object of my invention to provide a process for the recovery of terne metal from scruff, which shall be simple and economical and by means of which the percentage of recovery shall be greatly increased.

10 A further object of my invention is the provision of a process for the recovery of terne metal from scruff which shall greatly reduce the furnace reduction treatment heretofore practiced in prior art processes and which shall also 15 reduce the volatilization losses of metal.

As is well known, there are considerable losses of metal in plating processes and the metal in the form of prills, oxides and chlorides is mixed with iron scrap, sawdust, sweepings, and oil and 20 grease making up the scruff. The terne metal content of the scruff may vary from 20% to 50%.

It has heretofore been the practice to burn the combustible matter out of the scruff in a scruff 25 furnace, allowing the metal to melt and run out during the burning process, and then treat the remaining ash in a reverberatory furnace. The burning of the oil bearing scruff in this manner brings about such high temperatures that a considerable amount of the metal is volatilized off 30 and lost, and the furnace chimney is soon plugged with the deposited metal compounds.

In accordance with my invention, I first saponify or dissolve out the oily content of the 35 scruff with a caustic alkali solution, leaving a wet sludge containing the free metal, oxides, and a considerable amount of sawdust and other solid matter which is dried on an open dry plate. I may also employ in the alkali solution from 1% 40 to 2% of a petroleum distillate to aid in dissolving the oils and greases. As the water is driven off on the dry plate, the temperature of the dried mass increases and the combustible matter therein finally ignites, sweating the free metal 45 out of the mass and leaving an ash containing principally the oxides of the metal. This ash, after separation of metallic iron, is then treated in a reverberatory furnace with sufficient carbon, preferably in the form of anthracite, to reduce the oxides to metal. By this process I can 50 control the initial temperatures at which the metal is sweated out of the scruff and thus prevent losses and also reduce materially the amount of ash to be treated in the reverberatory furnace. I have found that the recovery of

metal is increased approximately 10% by my improved method.

In the accompanying drawing, the single figure is a flow sheet showing the steps in my improved process.

Referring to the drawing, I charge a heating and agitating tank 10 equipped with a stirrer 11 with one ton of scruff consisting principally of sweepings, greasy, oily sawdust, metal prills, oxides and chlorides. To this is added sufficient alkali to saponify the oils and greases, which amounts ordinarily to around 30 pounds of caustic soda, 70 gallons, or 560 pounds, of water, and approximately one gallon of a petroleum distillate to aid in dissolving the oil and grease out 15 of the sawdust and sweepings.

The heating and agitating tank is provided with suitable heating means, such as the gas burners 12, and the mixture is raised to the boiling temperature of the water while vigorously agitating to bring about the reaction between the caustic soda and the saponifiable oils. The soluble oil assists during this time in separating the heavier oils from the sawdust. The reaction should be complete in approximately 20 two hours. The saponified oils and separated greases rise to the surface of the mixture and are skimmed off from the surface. The remainder of the mixture is then drained through the valve 13 into the settling tank 14. The operation just described also dissolves out the zinc-ammonium chloride which accompanies the 25 scruff as an impurity.

The mixture drained into the settling tank 14 30 consists of the substances carried in solution by the alkaline liquor, the sawdust, oxides, and free metal content of the scruff. The mixture is allowed to settle for about twelve hours, whereupon the clear liquor is syphoned off to waste and the remaining solids shoveled out of the 35 settling tank on to an open drying plate 15, which is heated underneath. The heat drives off the moisture out of the mixture, and as the temperature rises, the sawdust ignites and slowly 40 burns, causing the metal to be sweated out. The drying plate is preferably on an incline so that the free metal runs off the lower end of the plate into a receptacle from whence it may be 45 cleaned by remelting, if necessary, and run into molds.

The dross, or ashes, resulting from the drying 50 step, is next passed through a magnetic separator 16 to remove the metallic iron, which may amount to as much as 6% of the original mass of scruff. The remaining dross or ashes, consisting princi- 55

pally of the oxides of the plating metal and amounting to only about 12% of the original charge of scruff, is sent to a reverberatory furnace. In this respect my improved process is a 5 distinct improvement over prior art processes known to me, in that the percentage of the scruff given expensive furnace treatment is greatly reduced.

In the furnace around 35 pounds of soda ash 10 and a sufficient amount of carbon to reduce the metal oxides, preferably in the form of rice anthracite, is added, and the temperature so regulated as to reduce the oxides to metal, which is recovered in the usual manner.

15 By means of my improved process I have, in actual practice, greatly reduced the cost of metal recovered, overcome the difficulty due to stoppage of flues, such as is encountered in a scruff furnace, and have increased the recovery of metal from the 20 scruff approximately 10%. While I have described my invention as being applicable to the recovery of terne metal, it will be obvious that it may be used in the recovery of other metals, for example, from the scruff and residues collected in 25 the tin plate process.

While I have shown my invention in but one form, it will be obvious to those skilled in the art that it is not so limited, but is susceptible of various changes and modifications, without departing

from the spirit thereof, and I desire, therefore, that only such limitations shall be placed thereupon as are imposed by the prior art or as are specifically set forth in the appended claims.

What I claim is:

1. The process of recovering tin and terne metal from scruff which comprises reacting the scruff with a hot alkali solution to saponify the saponifiable oils and greases therein, said solution containing around 1.5% of a soluble mineral oil, 10 separating scum and saponified matter from the solution, allowing the remaining solids to settle out of the solution and draining off the solution, drying and burning the said solids in open air to sweat out the free metal, separating metallic iron 15 from the resultant ash, and reducing the oxides in the remaining ash to metal.

2. The process of recovering tin and terne metal from scruff which comprises reacting the scruff with a hot alkali solution to saponify the 20 saponifiable oils and greases therein, separating scum and saponified matter from the solution, allowing the remaining solids to settle out of the solution and draining off the solution, drying and burning the said solids in open air to sweat out 25 the free metal, separating metallic iron from the resultant ash, and reducing the oxides in the remaining ash to metal.

WILLIAM J. BULLOCK.